

J. R. BILLINGS.

PURIFYING CAST IRON AND ELIMINATING OBJECTIONABLE GASES AND OXIDES.

APPLICATION FILED MAY 25, 1916. RENEWED AUG. 25, 1921.

1,412,077.

Patented Apr. 11, 1922.



*FIG. 2.*



Witnesses

*J. H. Baker.*

*FIG. 3.*



Inventor

*James R. Billings*

*Bynes, Tammes & Brickman*

Attorneys

# UNITED STATES PATENT OFFICE.

JAMES R. BILLINGS, OF CHICAGO, ILLINOIS, ASSIGNOR TO J. R. BILLINGS IRON & STEEL COMPANY, OF CHICAGO, ILLINOIS, A CORPORATION OF SOUTH DAKOTA.

## PURIFYING CAST IRON AND ELIMINATING OBJECTIONABLE GASES AND OXIDES.

1,412,077.

Specification of Letters Patent. Patented Apr. 11, 1922.

Application filed May 25, 1916, Serial No. 99,879. Renewed August 25, 1921. Serial No. 495,280.

To all whom it may concern:

Be it known that I, JAMES R. BILLINGS, a citizen of the United States, residing at Chicago, in the county of Cook and State of Illinois, have invented certain new and useful Improvements in Purifying Cast Iron and Eliminating Objectionable Gases and Oxides, of which the following is a specification.

10 My invention relates to the purification of crude pig iron, or iron having the characteristics of such crude pig metal, and has for its object to so treat the crude metal as to improve its qualities to such an extent 15 that the improved metal will be suitable for making castings of all kinds; will be capable of casting practically free from blow holes; can be worked by tools much more rapidly than the crude cast iron and will 20 have greater strength than before treatment.

I have discovered that the character of the gases, which are always found in metallic crude iron, has a material effect on the physical and mechanical properties of the iron, 25 and I have discovered that by removing, as far as possible, the hydrogen and oxygen and any undesirable excess of phosphorus, and by dissolving as far as possible, the carbonic oxide, that a pig iron which has been 30 obtained by the ordinary smelting method now in common use, i. e. by the use of a hot blast with coke as fuel,—can be transformed into an iron having, to a marked degree, the desirable properties of the best qualities of

35 charcoal pig iron, smelted in a blast furnace with a cold blast. In other words, I have found that it is quite possible to produce from ordinary pig iron, even of rather inferior grade, by a simple and expeditious 40 process, a high quality of pig iron corresponding to the high grade cold blast charcoal or Swedish grades of pig iron.

The method of introducing the purifying agents which I employ is in general like that 45 employed in my prior Patent No. 625,738, dated May 30, 1890; and the present invention may, to some extent, be regarded as an addition to or improvement on the method described in that patent.

50 In carrying out my process I prefer to use an apparatus such as is disclosed in the accompanying drawings, although any other suitable apparatus may be employed.

In the accompanying drawings, Fig. 1 is

an axial section view of a ladle and suitable 55 apparatus for introducing purifying material:

Fig. 2 is a plan view of the introducing mechanism pertaining to the ladle and shown in Fig. 1;

Fig. 3 is a perspective of a sheet metal cap.

1 designates a ladle, which may be of any usual and suitable type, 2 a platform constructed to extend above the ladle and provided with an aperture 3 through which the 65 introducing tube may be inserted, 4 the introducing tube as a whole, and 5 a supporting frame, conveniently taking the form of a box, through the lower end of which the introducing tube extends and to which it is 70 rigidly united, by screw threads as shown.

The frame 5 is detachably held in place on the platform by means of a set of hook-links 6; the arrangement being such that when a charge of metal is to be treated, after it has 75 been placed in the ladle, the introducing tube is lowered through the platform and into the molten mass, and the frame 5 then locked to the platform by the hook-links.

The introducing tube comprises a metal 80 tube 7 and an outer refractory covering 10 which covers so much of the tube as is liable to be inserted in the molten metal.

Within the tube 7 is arranged to reciprocate, an ejector plunger 18, the stem 19 of 85 which is in the form of a rack which extends upwardly through the frame 5 and meshes with a spur-gear 20 mounted on a crank shaft 21, journaled to extend transversely through the frame and conveniently 90 operated manually by means of a crank handle 22. A roller 23 journaled in a cross frame strip 5' just back of the rack 19 holds the latter in mesh with the gear. A tin or sheet iron cap 24 is provided, which is constructed to fit tightly upon the lower end of the introducing tube and serves to hold the charge of purifying material within the tube after it has been placed therein.

The process as carried out with the foregoing apparatus is substantially as follows:—A suitable batch of metal having been charged into the ladle, and the requisite amount of pulverulent material, such as hereinafter described, placed in the delivery 105 end of the introducing tube, and confined therein, by placing the cap 24 upon the end of the tube, the latter is lowered through

the platform into the metal and the frame made fast. As soon as the lower end of the tube is fairly within the molten metal the cap 24 will be melted off thus exposing the 5 container material to the action of the molten metal.

To ensure the removal of the hydrogen, I introduce into the molten metal by means 10 of the tube in the manner above described, a sufficient quantity of fluorspar in a com- minuted or finely divided state, from one to ten pounds of fluorspar per ton of molten pig iron being sufficient for this purpose, although it is to be understood that I do not 15 limit myself to any specific proportions.

In case the crude pig iron should contain more phosphorus than is regarded as desirable, the phosphorus content may readily be lowered by introducing into the molten 20 metal, through the above mentioned mechanical device, a sufficient quantity of preferably finely divided or comminuted sodium nitrate or other phosphorus-removing ingredients, one to ten pounds per ton of molten pig iron being used, although I do 25 not wish to be limited to these specific proportions. Instead of nitrate of soda there may be used a mixture of calcium carbonate or oxide and fluorspar, and it is, therefore, 30 quite possible to obtain the simultaneous removal of the hydrogen and any excess of phosphorus by properly proportioning the amount of added fluorspar.

Finely divided carbon may also be introduced, preferably after the other ingredients. The order in which the purifying 35 agents are added may be attained by placing in the introducing tube, first, the carbon, then the phosphorus-removing agent, 40 and then nearest the exit end, the hydrogen removing agent. All these operations can be so rapidly performed that the fluidity of the metal is not substantially lowered, and any loss of heat in the treatment for the 45 removal of hydrogen and phosphorus, can be compensated by the additional heat furnished by the combustion of carbonaceous fuel. The treatment above described has the added effect of practically freeing the molten metal from any oxide of iron and is also 50 effective in eliminating the sulfur by chemi-

cal reaction due to the high temperature produced.

It is desirable to cast the meal when treated by the above process into cold molds, 55 preferably made of iron, so that the metal as far as its content of retained gases is concerned, will be maintained as far as possible in the condition in which it is left by the treatment in the ladle.

The product resulting from the treatment above described is an iron of superior quality with its objectionable gases and oxides eliminated, and which is peculiarly soft and tough and suitable for making castings 60 which require machining or tooling. When remelted and used in foundry practice for making castings, this metal will cast sound and practically free from blow holes, will tool much faster than crude pig iron and is 70 much stronger than before treatment. It is also adapted for the valuable purpose of making malleable iron castings. The product also has to a marked degree the quality that when remelted in the cupola, it is in a 75 condition much hotter and more fluid than ordinary pig iron.

My method, therefore, enables the purification of crude pig iron either as it comes 80 from the blast furnace or as obtained by remelting mixtures of pig iron and scrap in the cupola, in such manner and with such results that it is adapted not only for making castings of all kinds, but is also a suitable 85 base for high grade iron and steel manufacture.

I claim:—

1. The improvement in the art of making iron which consists in introducing into the crude molten metal a hydrogen eliminating 90 agent, and a phosphorus-removing agent and then gradually and positively introducing into the body of the molten metal finely divided carbon.

2. The improvement in the art of making 95 iron which consists in gradually and positively passing downwardly into the crude molten metal, a finely divided hydrogen-eliminating agent, a phosphorus-removing agent, and finely divided carbon.

In testimony whereof I affix my signature.  
JAMES R. BILLINGS.